# EUROPEAN PATENT SPECIFICATION

(11) **EP 1 577 111 B1**
(45) Date of publication and mention of the grant of the patent: **28.02.2007**
(21) Application number: 05005635.7
(22) Date of filing: 15.03.2005
(51) Int. Cl.: B41M 5/36, B41C 1/10

(54) **Positive-type photosensitive composition**
Positiv arbeitende photoempfindliche Zusammensetzung
Composition photosensible de type positif

(30) Priority: 16.03.2004 JP 2004075119; 16.03.2004 JP 2004075121; 30.08.2004 JP 2004250843
(43) Date of publication of application: 21.09.2005
(73) Proprietor: FUJI PHOTO FILM CO., LTD., Minami-Ashigara-shi, Kanagawa (JP)
(72) Inventor: Watanabe, Kotaro, Yoshida-cho, Haibara-gun, Shizuoka-ken (JP); Kawauchi, Ikuo, Yoshida-cho, Haibara-gun, Shizuoka-ken (JP); Hatanaka, Yusuke, Yoshida-cho, Haibara-gun, Shizuoka-ken (JP)
(74) Representative: HOFFMANN EITLE

(56) References cited:
- EP-A- 1 262 318
- EP-A- 1 439 058
- EP-A- 1 462 251
- EP-A- 1 510 866
- US-A- 5 786 125

## Description

### Field of the Invention

The present invention relates to a positive-type photosensitive composition that increases its solubility in an aqueous alkaline solution by exposure to infrared rays. In particular it relates to a positive-type photosensitive composition useful as an image-recording layer for so-called direct-plate-making planographic printing plate precursors that allow direct plate-making by scanning an infrared laser based on digital signals from, for example, a computer.

### Description of the Related Art

Various photosensitive compositions have been used as visible image-forming materials and planographic printing plate materials. With the recent rapid progress in the development of lasers, especially in planographic printing, higher-output and smaller solid state and semiconductor lasers having emission wavelengths in the range from near-infrared to infrared region are becoming more easily accessible. When plate making is performed directly from digital data from, for example. a computer, these lasers play an important role as exposure-light sources.

Positive-type planographic printing plate precursors for infrared laser have an aqueous alkaline solution-soluble binder resin and an IR dye or the like, that absorbs light and generates heat, as the essential components. Planographic printing plates are produced from the precursors using the following mechanism. The IR. dye or the like therein functions as a solubilization inhibitor, substantially reducing the solubility of the binder resin, by interaction with the binder resin, in the unexposed regions (image regions). The binder resin dissolves in an alkaline developer in the exposed regions (non-image regions), because of the weakened interaction between the IR dye or the like and the binder resin, due to the heat generated.

However, the positive-type planographic printing plate precursors for infrared laser had the problem that the difference between the insolubility of binder resin in the unexposed regions (image regions) and the solubility thereof in the exposed regions (non-image regions) in the developer (hereinafter, referred to as solubility discrimination) was not large enough under various conditions of developing. Often this lead to variation in the quality of developed images, excessive or insufficient, depending on the conditions of developing.

To overcome this problem, a photosensitive composition wherein the major portion of the alkali-soluble resin is made of a novolak resin (e.g., European Patent Application Laid-Open No. 0823327A2) was proposed as the method for improving the solubility discrimination. The novolak resin in the unexposed region became less soluble in the developer, due to hydrogen bonding among phenolic hydroxyl groups, interaction with other additives contained in the photosensitive composition, or the like, and more soluble in the exposed region by the heat generated, improving the solubility discrimination. However, this resin still had the problem that the solubility discrimination was not really satisfactory, and also there was low developing stability (development latitude) for the conditions of use.

On the other hand, many compounds have been examined as solubilization inhibitors, and among them, onium salt-type solubilization inhibitors have been known to have very strong solubilization-inhibiting ability. However, although addition of a common onium salt compound was effective in improving the alkali resistance of the resin in the unexposed region, because of the enhanced solubilization-inhibiting potential, it still carried the problem of the deterioration in sensitivity caused by, for example, handling under white light. To overcome this problem, a new photosensitive composition containing a particular onium salt that has superior decomposition properties under light exposure was proposed (e.g., Japanese Patent Application Laid-Open (JP-A) No. 2002-278050). Although this onium salt showed better properties showing at the same time both high solubilization-inhibiting ability and high sensitivity, it became apparent that the salt caused a new problem. This problem was one of the deterioration in printing properties with time when, for example, an exposed plate was not developed immediately after exposure but developed after a certain period of time. The deterioration in printing properties with time after exposure is a serious problem in the plate-making process, requiring improvement. (Hereinafter, the degree of change in the printing properties over time after exposure is expressed by the term "post-exposure stability", and a greater degree of deterioration in printing properties is referred to as "inferior post-exposure stability".)

Recently, another photosensitive composition for improvement in development latitude was disclosed, containing a novolak resin and a vinyl polymer containing a particular amount of carboxyl groups and having a preadjusted solubility parameter (e.g., JP-A No. 2003-345014). The photosensitive composition is superior in coating forming properties and coating strength; further more the exposed regions thereof are rapidly dissolved in an aqueous alkaline solution. Thus the photosensitive composition is effective in improving the printing durability and the development latitude when used as a recording layer of a planographic printing plate precursor. However, the photosensitive composition still requires further improvement in the post-exposure stability when it is applied to a planographic printing plate precursor.

**EP-A-1 262 318** relates to a lithographic printing plate precursor comprising a support and an alkali-soluble resin-containing lower layer and a positive-working recording layer on the support. The recording layer contains an infrared absorbent and an alkali-soluble novolak resin containing xylenol as a structural unit.

**US-A-5 786 125** provides a light-sensitive lithographic printing plate comprising a support laminated with a light-sensitive layer and a silicone rubber layer, wherein the light-sensitive layer comprises a resol resin, a novolak resin, an infrared absorber and a compound which generates an acid upon heating.

**EP-A-1 439 058,** prior art according to Art. 54(3) EPC, relates to a positive planographic printing plate precursor comprising a hydrophilic support having a water-insoluble, alkali-soluble resin-containing lower layer and an image recording layer disposed thereon. The image recording layer contains a novolak resin containing phenol as a structural unit and a light-to-heat conversion agent.

**EP-A-1 462 251,** prior art according to Art. 54(3) EPC, discloses a method for producing a lithographic printing plate comprising exposing a positive-working pre-sensitized plate containing a substrate and an image recording layer to infrared radiation and subsequently developing the plate with an alkaline developing solution comprising an anionic and/or amphoteric surfactant. The image recording layer comprises a novolak resin containing xylenol as a monomer component and an infrared absorbing dye.

**EP-A-1 510 866,** prior art according to Art. 54(3) EPC, discloses an image recording material comprising an anodized aluminium support, an intermediate layer containing a polymer having a carboxylic acid group in a side chain thereof on the support and a photosensitive layer containing at least 50 wt.% of a novolak-type phenol resin and a photo-thermal conversion agent.

### SUMMARY OF THE INVENTION

The present invention has been made in view of the above circumstances and provides a positive-type photosensitive composition superior in sensitivity, greater in layer strength, and which readily releases the mutual interactions by infrared ray exposure, which is useful as a recording layer for positive-type planographic printing plate precursor.

The invention also provides a photosensitive composition superior in development latitude, sensitivity, and post-exposure stability, and useful as a recording layer for positive-type planographic printing plate precursors.

After intensive studies, the present inventors have found that the characteristics can be achieved by the means described below, and have achieved the invention.

A first aspect of the invention is a positive-type photosensitive composition comprising a novolak resin (A), an infrared absorbing agent (B), and a compound having a triarylsulfonium salt structure (C) in which the sum of Hammett values of substituents bonded to aryl skeletons is greater than 0.46.

In the invention, the term "compatible with heat mode" means that the precursor is compatible with recording by heat-mode exposure.

The definition of the heat-mode exposure in the invention will be described below in detail. As described in Hans-Joachim Timpe, IS&Ts NIP 15: 1999 International Conference on Digital Printing Technologies, p. 209, the disclosure of which is incorporated by reference herein, there are grossly two modes of processes from optical excitation of a light absorption material (e.g. dye) in a photosensitive material, via chemical or physical changes, to give image formation.

One is a so-called photon mode, wherein the optically excited light absorption material is inactivated by some photochemical interaction with another reactive material present in the photosensitive material (e.g., energy transfer or electron transfer), and the resulting activated reaction product triggers a chemical or physical change that is needed for the image formation described above.

Another is a so-called heat mode wherein the optically excited light absorption material is inactivated, emitting heat, this heat then triggers the chemical or physical change of the reactive material needed for the image formation described above.

There are also other special modes such as ablation wherein material is scattered explosively by locally concentrated light energy, and multi-photon absorption wherein a molecule absorbs multiple photons at the same time, but the description thereof is omitted here.

Exposure processes in the modes described before are referred to respectively as photon-mode exposure and heat-mode exposure. The technical difference between photon-mode exposure and heat-mode exposure is whether it is possible to add the energy of several exposure photons to the energy of the desired reaction.

For example, assume a case when a reaction is triggered by n photons. By the photon-mode exposure, which utilizes a photochemical interaction, the law of conservation of quantum energy and momentum prohibits the addition of the energy of several photons. In other words, in order to trigger a reaction, the following relation should be satisfied: $" Energy amount of a single photon > = reaction energy amount " .$

Whereas, in heat-mode exposure, which utilizes the heat converted from the photoenergy applied during photoexcitation, the addition of energy from several photons is allowed. Thus in this case, only the following relationship need be satisfied: $" Energy amount of n photon > = reaction energy amount " .$

However, the addition of the energy is restricted by thermal diffusion.

Namely, if the subsequent photoexcitation - inactivation process, generating heat, occurs before the removal of heat from the exposed region area (reactive area) by thermal diffusion, then heat certainly builds up, leading to an increase in the temperature of the area. However, if the subsequent heat generation process is delayed then there is an escape of heat, prohibiting accumulation of heat.

With heat-mode exposure the result is different between when high-energy light is irradiated for a short period and when low-energy light is irradiated for a long period, even if the total exposure energy is the same. The short-term irradiation of high-energy light is more advantageous for heat accumulation.

Of course, a similar phenomenon may be encountered due to the influence of the diffusion of reactive species even with photon-mode exposure, but practically this does not occur.

In terms of the properties of the photosensitive material, with photon mode the inherent sensitivity of photosensitive material (energy of the reaction required for image formation) remains constant even when the exposure power density (W/cm²) (energy density per unit period) varies, but the inherent sensitivity of the photosensitive material increases as the exposure power density increases with heat mode.

Accordingly, when these modes are compared in practice as image recording materials, with the necessary exposure times for maintaining the required productivity rates, photon-mode exposure photosensitive materials are inherently sensitive at a relatively low level (approximately 0.1 mJ/cm²), and can be made highly sensitive. However, the reaction inevitably occurs with photon-mode exposure, no matter how low the exposure intensity is, often leading to the problem of low-exposure background fogging in unexposed regions.

In contrast, with heat-mode exposure the reaction occurs only when the photosensitive material is irradiated at a certain exposure intensity or higher. As a result, considering the thermal stability of photosensitive materials, a photosensitive material normally having an inherent sensitivity of approximately 50 mJ/cm² can avoid the problem of the low-exposure background fogging.

In fact, photosensitive material require an exposure power density on the plate surface of 5,000 W/cm² or more, preferably 10,000 W/cm² or more, with heat-mode exposure. However, although not described here in detail, use of a high-power density laser of 5.0×10⁵ W/cm² or more is not favorable, as it causes ablation, resulting in problems such as staining of the light source.

In short, the invention provides an image-forming material useful for positive-type planographic printing plate precursors compatible with heat mode, superior in solubility discrimination, and favorable in post-exposure stability. Application of this image-forming material enables production of a positive-type planographic printing plate precursors superior in development latitude, permitting high-sensitivity recording, and with improved post-exposure stability.

### DETAILED DESCRIPTION OF THE INVENTION

Hereinafter, a first embodiment of the positive-type photosensitive composition according to the present invention (hereinafter, referred to simply as photosensitive composition) will be described in detail.

### First embodiment

The positive-type photosensitive composition according to the invention (present embodiment) characteristically contains a novolak resin (A), an infrared absorbing agent (B), and a compound having a triarylsulfonium salt structure (C) in which the sum of Hammett values of substituents bonded to aryl skeletons is greater than 0.46.

Constituent components of the photosensitive composition according to the invention will be described separately below.

### [Novolak resin (A)]

Examples of the novolak resins used in the invention include resins prepared by polycondensation of at least one phenol such as phenol, o-cresol, m-cresol, p-cresol, 2,5-xylenol, 3,5-xylenol, o-ethylphenol, m-ethylphenol, p-ethylphenol, propylphenol, n-butylphenol, tert-butylphenol, 1-naphthol, 2-naphthol, pyrocatechol, resorcinol, hydroquinone, pyrogallol, 1,2,4-benzenetriol, fluoroglycinol, 4,4'-biphenyldiol, or 2,2-bis(4'-hydroxyphenyl)propane, with at least one aldehydes such as formaldehyde, acetaldehyde, propionaldehyde, benzaldehyde, or furfural (formaldehyde may be substituted with paraformaldehyde and acetaldehyde with paraldehyde) or a ketone such as acetone, methylethylketone, or methylisobutylketone, for example, in the presence of an acid catalyst.

In the invention, favorable are polycondensation polymers from a phenol such as phenol, o-cresol, m-cresol, p-cresol, 2,5-xylenol, 3,5-xylenol, or resorcinol and an aldehyde or ketone such as formaldehyde, acetaldehyde, or propionaldehyde; in particular, polycondensation polymers from a mixed phenol containing m-cresol: p-cresol: 2,5-xylenol: 3,5-xylenol: resorcinol at a molar ratio of 40 to 100: 0 to 50: 0 to 20: 0 to 20: 0 to 20, or containing phenol: m-cresol: p-cresol at a molar ratio of 0 to 100: 0 to 70: 0 to 60 and formaldehyde are preferable.

The photosensitive composition according to the invention contains the sulfonium salt (C) described below as a solubilization inhibitor. Considering the interaction with the sulfonium salt, a polycondensation polymer from a mixed phenol containing m-cresol: p-cresol: 2,5-xylenol: 3,5-xylenol: resorcinol at a molar ratio of 70 to 100: 0 to 30: 0 to 20: 0 to 20: 0 to 20, or containing phenol: m-cresol: p-cresol at a molar ratio of 10 to 100: 0 to 60: 0 to 40 and formaldehyde is preferable as the novolak resin (A) in the invention.

The weight-average molecular weight of the novolak resin (A) as polystyrene, as determined by gel-permeation chromatography (hereinafter, referred simply as weight-average molecular weight) is preferably 500 to 20,000, still more preferably 1,000 to 15,000, and particularly preferably 3,000 to 12,000. When the weight-average molecular weight is in the range, the resin has a sufficiently high layer-forming capacity and a high alkali-solubility in the region exposed to infrared ray irradiation.

Alternatively, the content of novolak resin (A) in the photosensitive composition according to the invention is preferably in the range of 50 to 95%, more preferably in the range of 70 to 93%, and still more preferably, 75 to 85% by weight with respect to the total solid matters in the photosensitive layer composition, from the viewpoints of both surface layer-forming properties and resistance to alkaline developer.

### [Infrared absorbing agent (B)]

Infrared-absorbing dyes or pigments having an absorption maximum wavelength in the range of 760 nm to 1,200 nm are favorably used as the infrared absorbing agent (C) usable in the photosensitive composition according to the invention, from the viewpoint of compatibility with high-output lasers, i.e., readily available exposure-light sources.

The dyes may be commercially available ones and, for example, known ones described in publications such as "Dye Handbook" (edited by the Society of Synthesis Organic Chemistry, Japan, and published in 1970). Specific examples thereof include azo dyes, metal complex azo dyes, pyrazolone azo dyes, naphthoquinone dyes, anthraquinone dyes, phthalocyanine dyes, carbonium dyes, quinoneimine dyes, methine dyes, cyanine dyes, squalirium dyes, pyrylium dyes, metal thiolate complexes, oxonol dyes, diimonium dyes, aminium dyes, and croconium dyes.

Preferable examples of the dye include cyanine dyes described in JP-A Nos. 58-125246, 59-84356, 59-202829, and 60-78787; methine dyes described in JP-A Nos. 58-173696, 58-181690, and 58- 191595; naphthoquinone dyes described in JP-A Nos. 58-112793, 58-224793, 59-48187, 59-73996, 60-52940, and 60-63744; squalirium dyes described in JP-A No. 58-112792; and cyanine dyes described in GB Patent No. 434,875.

Other preferable examples of the dye include near infrared absorbing sensitizers described in U.S. Patent No. 5,156,938; substituted arylbenzo(thio)pyrylium salts described in U.S. Patent No. 3,881,924; trimethinethiapyrylium salts described in JP-A No. 57-142645 (U.S. Patent No. 4,327,169); pyrylium type compounds described in JP-A Nos. 58-181051, 58-220143, 59-41363, 59-84248, 59-84249, 59-146063, and 59-146061; cyanine dyes described in JP-A No. 59-216146; pentamethinethiopyrylium salts described in U.S. Patent No. 4,283,475; and pyrylium compounds described in Japanese Patent Application Publication (JP-B) Nos. 5-13514 and 5-19702.

Additional preferable examples of the dye include near infrared absorbing dyes represented by formulae (I) and (II) as described in U.S. Patent No. 4,756,993.

Among these dyes, particularly preferable are cyanine dyes, phthalocyanine dyes, oxonol dyes, squalirium dyes, pyrylium salts, thiopyrylium dyes, and nickel thiolate complexes. Dyes represented by the following general formulae (a) to (e) are also preferable since such dyes are excellent in terms of photothermal conversion efficiency. The cyanine dyes represented by the following general formula (S-1) are most preferable for the following reason: when the dyes are used in the photosensitive composition of the invention, the dyes manifest a high degree of interaction with the alkali-soluble resin, and the dyes are also excellent in terms of stability and economy.

### General formula (S-1)

In general formula (S-1), X¹ represents a hydrogen atom, a halogen atom, -NPh₂, X²-L¹ (wherein X² represents an oxygen atom or a sulfur atom, L' represents a hydrocarbon group having 1 to 12 carbon atoms, an aromatic cyclic group having a heteroatom, or a hydrocarbon group containing a heteroatom and having 1 to 12 carbon atoms, and the heteroatom referred to herein is N, S, O, a halogen atom, or Se), or a group represented by the following: wherein Xa⁻ has the same definition as Za⁻, which will be described at a later time, and R^{a} represents a substituent selected from a hydrogen atom, an alkyl group, an aryl group, a substituted or unsubstituted amino group, or a halogen atom;

R¹ and R² each independently represents a hydrocarbon group having 1 to 12 carbon atoms, and from the viewpoint of the storage stability of the photosensitive composition of the invention when it is used in a coating solution for forming a recording layer of a planographic printing plate precursor, it is preferable that R¹ and R² each independently represents a hydrocarbon group having 2 or more carbon atoms, and more preferably R¹ and R² are bonded to each other to form a 5-membered or 6-membered ring.

Ar¹ and Ar², which may be the same or different, each represent an aromatic hydrocarbon group which may have a substituent. Preferable examples of the aromatic hydrocarbon group include benzene and naphthalene rings. Preferable examples of the substituent include hydrocarbon groups having 12 or less carbon atoms, halogen atoms, and alkoxy groups having 12 or less carbon atoms.

Y¹ and Y², which may be the same or different, each represents a sulfur atom, or a dialkylmethylene group having 12 or less carbon atoms.

R³ and R⁴, which may be the same or different, each represents a hydrocarbon group which has 20 or less carbon atoms and may have a substituent. Preferable examples of the substituent include alkoxy groups having 12 or less carbon atoms, a carboxyl group, and a sulfo group. R⁵, R⁶, R⁷ and R⁸, which may be the same or different, each represents a hydrogen atom, or a hydrocarbon group having 12 or less carbon atoms, and since the raw materials thereof can easily be obtained, each preferably represents a hydrogen atom.

Za⁻ represents a counter anion. However, in a case where the cyanine dye represented by general formula (S-1) has an anionic substituent in the structure thereof and there is accordingly no need to neutralize electric charges in the dye, Za⁻ is not required. From the viewpoint of the storage stability of the recording layer coating solution, Za⁻ is preferably an ion of a halogen, perchlorate, tetrafluroborate, hexafluorophosphate, carboxylate or sulfonate. From the viewpoints of compatibility of the dye with the alkali-soluble resin and solubility in the coating solution, Za⁻ is preferably a halogen ion, or an organic acid ion such as a carboxylic acid ion or sulfonic acid ion, more preferably a sulfonic acid ion, and even more preferably an arylsulfonic acid ion.

Specific examples of the cyanine dye represented by general formula (S-1), and which can be preferably used in the invention, include dyes in JP-A No. 2001-133969 (paragraphs [0017] to [0019]), JP-A No. 2002-40638 (paragraphs [0012] to [0038]), and JP-A No. 2002-23360 (paragraphs [0012] to [0023]), as well as dyes illustrated below.

In general formula (S-2), L represents a methine chain having 7 or more conjugated carbon atoms, and the methine chain may have one or more substituent. The substituents may be bonded to each other to form a cyclic structure. Zb⁺ represents a counter cation. Preferable examples of the counter cation include ammonium, iodonium, sulfonium, phosphonium and pyridinium ions, and alkali metal cations (such as Ni⁺, K⁺ and Li⁺).

R⁹ to R¹⁴ and R¹⁵ to R²⁰ each independently represents a substituent selected from hydrogen atom, halogen atom, and cyano, alkyl, aryl, alkenyl, alkynyl, carbonyl, thio, sulfonyl, sulfinyl, oxy and amino groups; or a substituent obtained by combining two or three from among these substituents. Two or three out of R⁹ to R¹⁴ and R¹⁵ to R²⁰ may be bonded to each other to form a cyclic structure.

A dye wherein L in general formula (S-2) represents a methine chain having 7 conjugated carbon atoms, and each of R⁹ to R¹⁴ and R¹⁵ to R²⁰ represents a hydrogen atom, is preferable since such a dye can be easily obtained and exhibits advantageous effects.

Specific examples of the dye represented by general formula (S-2), and which can be preferably used in the invention, are illustrated below.

In general formula (S-3), Y³ and Y⁴ each independently represent an oxygen, sulfur, selenium or tellurium atom; M represents a methine chain having 5 or more conjugated carbon atoms; R²¹ to R²⁴ and R²⁵ to R²⁸, which may be the same or different, each represents a hydrogen or halogen atom, or a cyano, alkyl, aryl, alkenyl, alkynyl, carbonyl, thio, sulfonyl, sulfinyl, oxy or amino group; and Za- represents a counter anion, and has the same meaning as Za⁻ in general formula (S-1).

Specific examples of the dye which is represented by general formula (S-3) and which can be preferably used in the invention, are illustrated below.

In general formula (S-4), R²⁹ to R³¹ each independently represents a hydrogen atom, an alkyl group or an aryl group; R³³ and R³⁴ each independently represents an alkyl group, a substituted oxy group, or a halogen atom; n and m each independently represents an integer of 0 to 4; and R²⁹ and R³⁰, or R³¹ and R³² may be bonded to each other to form a ring, or R²⁹ and/or R³⁰ may be bonded to R³³ to form a ring and R³¹ and/or R³² may be bonded to R³⁴ to form a ring. When plural R^{33,}s and R^{34,}s are present, R^{33,}s may be bonded to each other to form a ring, or R^{34,}s may be bonded to each other to form a ring.

X² and X³ each independently represents a hydrogen atom, an alkyl group or an aryl group, and at least one of X² and X³ represents a hydrogen atom or an alkyl group.

Q represents a trimethine group or a pentamethine group which may have a substituent, and may be combined with an bivalent linking group to form a cyclic structure. Zc⁻ represents a counter anion and has the same meanings as Za⁻ in general formula (S-1).

Specific examples of the dye represented by general formula (S-4) and which can be preferably used in the invention, are illustrated below.

In general formula (S-5), R³⁵ to R⁵⁰ each independently represents a hydrogen or halogen atom, or a cyano, alkyl, aryl, alkenyl, alkynyl, hydroxyl, carbonyl, thio, sulfonyl, sulfinyl, oxy or amino group, or an onium salt structure, each of which may have a substituent; M represents two hydrogen atoms, a metal atom, a halo metal group, or an oxy metal group. Examples of the metal contained therein include atoms in IA, IIA, IIIB and IVB groups in the periodic table, transition metals in the first, second and third periods therein, and lanthanoid elements. Among these examples, preferable are copper, magnesium, iron, zinc, cobalt, aluminum, titanium, and vanadium.

Specific examples of the dye represented by general formula (S-5) and which can be preferably used in the invention, are illustrated below.

The pigment used as the infrared absorbent in the invention may be a commercially available pigment or a pigment described in publications such as Color Index (C.I.) Handbook, "Latest Pigment Handbook" (edited by Japan Pigment Technique Association, and published in 1977), "Latest Pigment Applied Technique" (by CMC Publishing Co., Ltd. in 1986), and "Printing Ink Technique" (by CMC Publishing Co., Ltd. in 1984).

Examples of the pigment include black pigments, yellow pigments, orange pigments, brown pigments, red pigments, purple pigments, blue pigments, green pigments, fluorescent pigments, metal powder pigments, and polymer-bonded dyes. Specifically, the following can be used: insoluble azo pigments, azo lake pigments, condensed azo pigments, chelate azo pigments, phthalocyanine pigments, anthraquinone pigments, perylene and perynone pigments, thioindigo pigments, quinacridone pigments, dioxazine pigments, isoindolinone pigments, quinophthalone pigments, dyeing lake pigments, azine pigments, nitroso pigments, nitro pigments, natural pigments, fluorescent pigments, inorganic pigments, and carbon black. Among these pigments, carbon black is preferable.

These pigments may be used with or without surface treatment. Examples of surface treatment include a method of coating the surface of the pigments with resin or wax; a method of adhering a surfactant onto the surface; and a method of bonding a reactive material (such as a silane coupling agent, an epoxy compound, or a polyisocyanate) to the pigment surface. The surface treatment methods are described in "Nature and Application of Metal Soap" (Saiwai Shobo), "Printing Ink Technique" (by CMC Publishing Co., Ltd. in 1984). And "Latest Pigment Applied Technique" (by CMC Publishing Co., Ltd. in 1986.

The particle size of the pigment is preferably from 0.01 to 10 µm, more preferably from 0.05 to 1 µm, and even more preferably from 0.1 to 1 µm. When a particle size is within the preferable range, a superior dispersion stability of the pigment in the photosensitive composition can be obtained, whereby, when the photosensitive composition of the invention is used for a recording layer of the photosensitive printing plate precursor, it is possible to form a homogeneous recording layer.

The method for dispersing the pigment may be a known dispersing technique used to produce ink or toner. Examples of a dispersing machine, which can be used, include an ultrasonic disperser, a sand mill, an attriter, a pearl mill, a super mill, a ball mill, an impeller, a disperser, a KD mill, a colloid mill, a dynatron, a three-roll mill, and a pressing kneader. Details are described in "Latest Pigment Applied Technique" (by CMC Publishing Co., Ltd. in 1986).

From the viewpoints of sensitivity, uniformity of the film to be formed and durability, the pigment or dye can be added to the photosensitive composition in a ratio of 0.01 to 50%, preferably 0.1 to 10%, and more preferably 0.5 to 10% (in the case of the dye) or 0.1 to 10% (in the case of pigment) by mass, relative to the total solid contents which constitute the photosensitive composition.

### [Sulfonium salt (C)]

The photosensitive composition according to the invention contains a compound having a triarylsulfonium salt structure (c) in which the sum of Hammett values of substituents bonded to aryl skeletons is greater than 0.46.

Triarylsulfonium salt (C) contains a strong acid residue Z⁻ as a counter anion. Specific examples thereof include halide ions, perchlorate ion, hexafluorophosphate ion, tetrafluoroborate ion, sulfonate ion, sulfinate ion, thiosulfonate ion, and sulfate ion; and perchlorate ion, hexafluorophosphate ion, tetrafluoroborate ion, sulfonate ion, and sulfinate ion are preferable from the viewpoint of stability.

The sulfonium salt (C) provides stability of non-image areas due to its main skeleton, and provides good removal of exposed regions (the good removal property is provided because decomposability of the triarylsulfonium salt by exposure is enhanced by acceleration of thermal decomposition or lowering of potential), thereby achieving effective suppression of staining.

### - Triarylsulfonium Salt Structure -

Compounds having a triarylsulfonium salt structure are known, for example, as polymerization initiators, and can be easily synthesized according to methods described, for example, in: J. Amer. Chem. Soc. Vol. 112 (16), 1990, pp. 6004-6015; J. Org. Chem., 1988, pp. 5571-5573; WO 02/081439A1; and EP 1113005.

### - Substituent Bonded to Aryl Skeleton -

As the substituents bonded to the aryl skeletons of the triarylsulfonium salt structure an electron attracting substituent is preferable. The sum of Hammett values of the electron attracting substituents bonded to the three aryl skeletons needs to be greater than 0.46, and preferably is greater than 0.60. If the sum of Hammett values is 0.46 or less, a sufficient anti-scumming property cannot be provided.

The Hammett value represents a degree of an electron attracting property of a cation having a triarylsulfonium salt structure, and there is no upper limit specified in view of provision of high sensitivity. However, in view of reactivity and stability, the Hammett value is preferably greater than 0.46 and less than 4.0, more preferably is greater than 0.50 and less than 3.5, and particularly preferably is greater than 0.60 and less than 3.0.

It should be noted that, as the Hammett values in this invention, values described in "Chemistry Seminar 10 Hammett Rule - Structure and Reactivity -" (edited by Naoki Inamoto, published by Maruzen, 1983) are used.

Examples of the electron attracting substituent introduced in the aryl skeleton include a trifluoromethyl group, a halogen atom, an ester group, a sulfoxide group, a cyano group, an amide group, a carboxyl group and a carbonyl group. Hammett values of these substituents are as follows: trifluoromethyl group (-CF₃, m: 0.43, p: 0.54); halogen atom [for example, -F (m:0.34, p:0.06), -Cl (m:0.37, p: 0.23), -Br (m:0.39, p:0.23), -I (m:0.35, p:0.18)]; ester group (for example, -COCH₃, o: 0.37, p: 0.45); sulfoxide group (for example, -SOCH₃, m: 0.52, p: 0.45); cyano group (-CN, m: 0.56, p: 0.66), amide group (for example, -NHCOCH₃, m: 0.21, p: 0.00); carboxyl group (-COOH, m: 0.37, p: 0.45); carbonyl group (-CHO, m: 0.36, p:(0.43)). The descriptions contained in the parentheses represent positions for introducing the substituents into the aryl skeleton and Hammett values thereof, and "(m: 0.50)", for example, represents that the Hammett value of the relevant substituent introduced in the meta-position is 0.50.

Among these substituents, nonionic substituents such as a halogen atom and an alkyl halide group are preferable in view of hydrophobicity. Among nonionic substituents, -Cl is preferable in view of reactivity, and -F, -CF₃, -Cl and -Br are preferable in view of providing hydrophobicity to the film.

These substituents may be introduced in any one of three aryl skeletons in the triarylsulfonium salt structure, or may be introduced into two or more aryl skeletons thereof. Further, one or plural substituents may be introduced into the individual three aryl skeletons. Positions for substitution and the number of substituents are not particularly specified as long as the sum of the Hammett values of the substituents introduced into the aryl skeletons is greater than 0.46. For example, one substituent having a particularly large Hammett value (a Hammett value exceeding 0.46 on its own) may be introduced into one of the aryl skeletons of the triarylsulfonium salt structure, or alternatively, plural substituents may be introduced so that the sum of the Hammett values thereof exceeds 0.46.

As described above, the Hammett values of the substituents vary depending on positions where they are introduced, and therefore, the sum of the Hammett values of the triarylsulfonium salt initiator will be determined according to the types of substituents, positions for introduction and the number of introduced substituents.

It should be noted that a Hammett side is usually represented by m-position, p-position, however, in the invention, as an indication of the electron attracting property, an effect of a substituent at o-position is considered as the same as that at p-position in calculation.

Among the specific sulfonium salts, a sulfonium salt substituted at three positions by chloro groups is most preferable, and specifically, a sulfonium salt having a triarylsulfonium salt structure where -Cl is introduced into each of three aryl skeletons is preferable.

Examples of a counter anion of the sulfonium salt preferably usable, in view of stability, in the invention include sulfonic acid anion, benzoylformic acid anion, PF₆⁻, BF₄⁻, ClO₄⁻, carboxylic acid anion, sulfinic acid anion, sulfuric acid anion, borate anion, halogen anion, phosphoric acid anion, phosphonic acid anion, phosphinic acid anion, active imide anion, polymeric sulfonic acid anion and polymeric carboxylic acid anion. It should be noted that a hydrophilicity/hydrophobicity parameter log P of the counter anion is preferably less than 2, in view point of effective suppression of scumming in the non-image areas, which is achieved by the recording layer being quickly removed and dispersed in a developing solution to expose a hydrophilic surface of a support with no residual film remaining thereon. More preferably, a value of log P is in a range from -1 to 1 in view of alkali developability and a film forming property.

Here, log P of the anion refers to log P of the log P of an acidic compound when the anion exists in the form of the acidic compound. In the invention, the hydrophilicity/hydrophobicity parameter log P of the anion moiety means a common logarithm of a partition coefficient P of the acidic compound including the anion moiety, and is a physical property value representing, as a quantitative value, how a certain organic compound is distributed at equilibrium in a two-phase system containing an oil (typically, 1-octanol) and water, which can be found by the following equation: $log P = log ( Coil / Cwater ) ,$
where Coil represents a mol concentration in oil phase and Cwater represents a mol concentration in water phase. A larger absolute value of log P in a positive direction from 0 represents a greater solubility in oil, whereas a larger absolute value of log P in a negative direction from 0 represents a greater solubility in water. There is a negative correlation between this value and a water-solubility of an organic compound, and this value is widely used as a parameter for estimating hydrophilicity/hydrophobicity of a compound. In principle, log P values are empirically measured in a distribution experiment. However, since this experiment is complicated, log P values value are usually obtained using an on-line database containing actual measurement values or calculation software for estimating log P values from structural formulae. The invention uses values calculated by using a log P value estimating program: CLOGP, developed by MedChem Project by C. Hansch, A. Leo, et al. from Pomona College, U.S.A. and Biobyte Corporation (CLOGP program: algorithm = 4.01, fragment database = 17, incorporated into a system: PCModels (ver. 1.02) provided by Daylight Chemical Information Systems, Inc.).

Examples of the compound having a triarylsulfonium salt structure in which the sum of Hammett values of substituents bonded to aryl skeletons is greater than 0.46 are listed below, but the invention is not restricted thereto:

The sulfonium salt (C) for use in the invention preferably has a maximum absorption wavelength of 400 nm or less and more preferably 360 nm or less. By bringing the absorption maximum wavelength into the ultraviolet region in this manner, it becomes possible to handle the photosensitive composition under white light.

The sulfonium salts (C) according to the invention may be used alone or in combination of two or more. When the photosensitive composition according to the invention is applied to a recording layer of planographic printing plate precursor, these sulfonium salts (C) may be added into the same layer together with other components or into another layer separately therefrom.

The sulfonium salts (C) favorably used in the invention include those containing a sulfonate or carboxylate anion as the counter anion.

The sulfonium salt (C) according to the invention may be added in an amount of 0.1 to 50% by weight, preferably 0.5 to 40% by weight, and particularly preferably 1 to 30% by weight with respect to the total solid matter in photosensitive composition from the viewpoints of sensitivity and elimination of interaction.

### [Other components]

Besides the essential components above, the photosensitive composition according to the invention may further contain other components as needed. Examples thereof include thermal degradable compounds such as onium salts, o-quinone diazide compounds, aromatic sulfone compounds, aromatic sulfonic ester compounds, and the like, and combined use of a material (thermally decomposable solubilization inhibitor) that practically reduces the solubility of alkali-soluble resin when not decomposed, is preferable for further reducing the solubilization thereof in the image region into the developer.

### [Onium salt]

Examples of the onium salts which are used as the other component in the photosensitive composition according to the invention include diazonium salts, ammonium salts, phosphonium salts, iodonium salts, selenonium salts, arsonium salts, and the like.

Preferable examples of the onium salt used in the invention include diazonium salts described in S. I. Schlesinger, Photogr. Sci. Eng., 18, 387 (1974), T. S. Bal et al., Polymer, 21, 423 (1980), and JP-A No. 5-158230; ammonium salts described in U.S. Patent Nos. 4,069,055 and 4,069,056, and JP-A No. 3-140140; phosphonium salts described in D. C. Necker et al., Macromolecules, 17, 2468 (1984), C. S. Wen et al., Teh, Proc. Conf. Rad. Curing ASIA, p478 Tokyo, Oct (1988), and U.S. Patent Nos. 4,069,055 and 4,069,056; iodonium salts described in J. V. Crivello et al., Macromolecules, 10 (6), 1307 (1977), Chem. & Eng. News, Nov. 28, p31 (1988), EP No. 104,143, U.S. Patent Nos. 5,041,358 and 4,491,628, and JP-A Nos. 2-150848 and 2-296514; sulfonium salts described in J. V. Crivello et al., Polymer J. 17, 73 (1985), J. V. Crivello et al., J. Org. Chem., 43, 3055 (1978), W. R. Watt et al., J. Polymer Sci., Polymer Chem. Ed., 22, 1789 (1984), J. V. Crivello et al., Polymer Bull., 14, 279 (1985), J. V. Crivello et al., Macromolecules, 14 (5), 1141 (1981), J. V. Crivello et al., J. Polymer Sci., Polymer Chem. Ed., 17, 2877 (1979), EP Nos. 370,693, 233,567, 297,443 and 297,442, U.S. Patent Nos. 4,933,377, 3,902,114, 5,041,358, 4,491,628, 4,760,013, 4,734,444 and 2,833,827, and DE Patent Nos. 2,904,626, 3,604,580 and 3,604,581; selenonium salts described in J. V. Crivello et al., Macromolecules, 10 (6), 1307 (1977), J. V. Crivello et al., J. Polymer Sci., Polymer Chem. Ed., 17, 1047 (1979); arsonium salts described in C. S. Wen et al., and The Proc. Conf. Rad. Curing ASIA, p478, Tokyo, Oct(1988).

Among such onium salts, diazonium salts are particularly preferable. The diazonium salts disclosed in the JP-A No. 5-158230 are the most preferable.

Examples of the counter ion of the onium salt include tetrafluoroboric acid, hexafluorophosphoric acid, triisopropylnaphthalenesulfonic acid, 5-nitro-o-toluenesulfonic acid, 5-sulfosalicylic acid, 2,5-dimethylbenzenesulfonic acid, 2,4,6-trimethylbenzenesulfonic acid, 2-nitrobenzenesulfonic acid, 3-chlorobenzenesulfonic acid, 3-bromobenzenesulfonic acid, 2-fluorocaprylnaphthalenesulfonic acid, dodecylbenzenesulfonic acid, 1-naphthol-5-sulfonic acid, 2-methoxy-4-hydroxy-5-benzoyl-benzenesulfonic acid, and p-toluenesulfonic acid. Among these examples, hexafluorophosphoric acid, and alkylaromatic sulfonic acids such as triisopropylnaphthalenesulfonic acid and 2,5-dimethylbezenesulfonic acid are particularly preferable.

The amount of the onium salt added is preferably in the range of 0.1 to 10%, still more preferably 0.1 to 5%, and particularly preferably 0.1 to 2% by weight with respect to the total solid matter in the image-recording layer.

These onium salts may be used alone or as a mixture of several salts.

### [o-Quinone diazide compound]

o-Quinone diazide compound for use in the photosensitive composition according to the invention is, for example, a compound having at least one o-quinone diazide group that becomes more alkali soluble by thermal decomposition, and such compounds in various structures may be used. Namely, o-quinone diazide makes the photosensitive composition more soluble by thermal decomposition, both by reducing the solubilization-inhibiting potential of novolak resin (A) and specific alkali-soluble resin (B) and converting itself to an alkali-soluble material. Examples of the o-quinone diazide compounds for use in the invention include the compounds described on pp. 339 to 352 of "Light Sensitive Systems" (J. Corsair Ed., John Wiley & Sons. Inc.), and in particular, sulfonic esters or sulfonic acid amides of the o-quinone diazides, which are prepared in reaction with various aromatic polyhydroxy compounds or aromatic amino compounds, are favorable. In addition, the esters from benzoquinone-(1,2)-diazido-sulfonylchloride or naphthoquinone-(1,2)-diazido-5-sulfonylchloride and a pyrogallol-acetone resin described in JP-B No. 43-28403, and the esters from benzoquinone-(1,2)-diazido-sulfonylchloride or naphthoquinone-(1,2)-diazido-5-sulfonylchloride and a phenol-formaldehyde resin described in U.S. Patent Nos. 3,046,120 and 3,188,210 are also favorably used.

Additional preferable examples include an ester made from naphthoquinone-(1,2)-diazide-4-sulfonic acid chloride and phenol-formaldehyde resin or cresol-formaldehyde resin; and an ester made from naphthoquinone-(1,2)-diazide-4-sulfonic acid chloride and pyrogallol-acetone resin.

Other useful o-quinonediazide compounds are reported in unexamined or examined patent documents, examples of which include JP-A Nos. 47-5303, 48-63802, 48-63803, 48-96575, 49-38701 and 48-13354, JP-B No. 41-11222, 45-9610 and 49-17481, U.S. Patent Nos. 2,797,213, 3,454,400, 3,544,323, 3,573,917, 3,674,495 and 3,785,825, GB Patent Nos. 1,227,602, 1,251,345, 1,267,005, 1,329,888 and 1,330,932, and DE Patent No. 854,890.

The amount of the o-quinone diazide compound added is preferably in the range of 0 to 10%, still more preferably 0 to 5%, and particularly preferably 0 to 2% by weight with respect to the total solid matter in photosensitive composition.

These o-quinone diazide compounds may be used alone or as a mixture of several compounds.

The amount of the thermally decomposable solubilization inhibitors excluding the onium salt and o-quinone diazide compound above is preferably 0 to 5%, still more preferably 0 to 2, and particularly preferably 0.1 to 1.5% by weight with respect to the total solid matters in photosensitive composition.

### [Other additives]

In order to enhance sensitivity, the photosensitive composition may also contain a cyclic acid anhydride, a phenolic compound, or an organic acid.

Examples of cyclic acid anhydride include phthalic anhydride, tetrahydrophthalic anhydride, hexahydrophthalic anhydride, 3,6-endooxy-Δ4-tetrahydrophthalic anhydride, tetrachlorophthalic anhydride, maleic anhydride, chloromaleic anhydride, α-phenylmaleic anhydride, succinic anhydride, and pyromellitic anhydride which are described in U.S. Patent No. 4,115,128.

Examples of phenolic compound include bisphenol A, p-nitrophenol, p-ethoxyphenol, 2,4,4'-trihydroxybenzophenone, 2,3,4-trihydroxybenzophenone, 4-hydroxybenzophenone, 4,4',4"-trihydroxytriphenylmethane, 4,4',3",4"-tetrahydroxy-3,5,3',5'-tetramethyltriphenylmethane.

Examples of the organic acid include sulfonic acids, sulfonic acids, alkylsulfuric acids, phosphonic acids, phosphates, and carboxylic acids, which are described in JP-A No. 60-88942 or 2-96755. Specific examples thereof include p-toluenesulfonic acid, dodecylbenzenesulfonic acid, p-toluenesulfinic acid, ethylsulfuric acid, phenylphosphonic acid, phenylphosphinic acid, phenyl phosphate, diphenyl phosphate, benzoic acid, isophthalic acid, adipic acid, p-toluic acid, 3,4-dimethoxybenzoic acid, phthalic acid, terephthalic acid, 4-cyclohexene-1,2-dicarboxylic acid, erucic acid, lauric acid, n-undecanoic acid, and ascorbic acid.

When the cyclic acid anhydride, the phenol or the organic acid is added to a recording layer of a planographic printing plate precursor, the ratio thereof in the recording layer is preferably from 0.05 to 20%, more preferably from 0.1 to 15%, and even more preferably from 0.1 to 10% by mass.

When the photosensitive composition according to the invention is used in a recording layer coating solution for a planographic printing plate precursor, in order to enhance stability in processes which affect conditions of developing, the following can be added: nonionic surfactants as described in JP-A Nos. 62-251740 and 3-208514; amphoteric surfactants as described in JP-A Nos. 59-121044 and 4-13149; siloxane compounds as described in EP No. 950517; and copolymers made from a fluorine-containing monomer as described in JP-A No. 11-288093.

Specific examples of nonionic surfactants include sorbitan tristearate, sorbitan monopalmitate, sorbitan trioleate, monoglyceride stearate, and polyoxyethylene nonyl phenyl ether. Specific examples of amphoteric surfactants include alkyldi(aminoethyl)glycine, alkylpolyaminoethylglycine hydrochloride, 2-alkyl-N-carboxyethyl-N-hydroxyethylimidazolinium betaine and N-tetradecyl-N,N'-betaine type surfactants (trade name: "Amolgen K", manufactured by Dai-ichi Kogyo Seiyaku Co., Ltd.).

The siloxane compounds are preferably block copolymers made from dimethylsiloxane and polyalkylene oxide. Specific examples thereof include polyalkylene oxide modified silicones (trade names: DBE-224, DBE-621, DBE-712, DBE-732, and DBE-534, manufactured by Chisso Corporation; trade name: Tego Glide 100, manufactured by Tego Co., Ltd.).

The content of the nonionic surfactant and/or the amphoteric surfactant in the photosensitive composition is preferably from 0.05 to 15% by mass, and more preferably from 0.1 to 5% by mass.

To the photosensitive composition of the invention may be added a printing-out agent for obtaining a visible image immediately after the photosensitive composition of the invention has been heated by exposure to light, or a dye or pigment as an image coloring agent.

A typical example of a printing-out agent is a combination of a compound which is heated by exposure to light, thereby emitting an acid (an optically acid-generating agent), and an organic dye which can form salts (salt formable organic dye).

Specific examples thereof include combinations of an o-naphthoquinonediazide-4-sulfonic acid halogenide with a salt-formable organic dye, described in JP-A Nos. 50-36209 and 53-8128; and combinations of a trihalomethyl compound with a salt-formable organic dye, described in each of JP-A Nos. 53-36223, 54-74728, 60-3626, 61-143748, 61-151644 and 63-58440.

The trihalomethyl compound is classified into an oxazol compound or a triazine compound. Both of the compounds provide excellent in stability over the passage of time and produce a vivid printed-out image.

As-the-image coloring agent, a dye different from the above-mentioned salt-formable organic dye may be used. Preferable examples of such a dye, and of the salt-formable organic dye, include oil-soluble dyes and basic dyes.

Specific examples thereof include Oil yellow #101, Oil Yellow #103, Oil Pink #312, Oil Green BG, Oil Blue BOS, Oil Blue #603, Oil Black BY, Oil Black BS, and Oil Black T-505 (each of which is manufactured by Orient Chemical Industries Ltd.); Victoria Pure Blue, Crystal Violet (CI42555), Methyl Violet (CI42535), Ethyl Violet, Rhodamine B (CI145170B), Malachite Green (CI42000), and Methylene Blue (CI52015).

Dyes described in JP-A No. 62-293247 are particularly preferable. These dyes may be added to the photosensitive composition at a ratio of 0.01 1 to 10% by mass, and preferably 0.1 to 3% by mass, relative to the total solid contents therein.

Whenever necessary, a plasticizer may be added to the photosensitive composition of the invention to give flexibility to a coating film made from the composition. Examples of the plasticizer include oligomers and polymers of butyl phthalyl, polyethylene glycol, tributyl citrate, diethyl phthalate, dibutyl phthalate, dihexyl phthalate, dioctyl phthalate, tricresyl phosphate, tributyl phosphate, trioctyl phosphate, tetrahydrofurfuryl olete, and acrylic acid and methacrylic acid.

In addition to the above, the following may be appropriately added to the composition, depending on the objective: an epoxy compound; a vinyl ether; a phenol compound having a hydroxymethyl group and a phenol compound having an alkoxymethyl group, described in JP-A No. 8-276558; and a cross-linkable compound having an effect of suppressing dissolution in an alkali, described in JP-A No. 11-160860, and which was previously proposed by the present inventors.

The photosensitive composition according to the invention can be applied to various recording materials in various applications such as planographic printing plate precursor, color-proof materials, and display material, by dissolving the respective components in a suitable solvent and applying the solution onto a support. In particular, it is useful as a heat mode-compatible positive-type planographic printing plate precursor that allows direct plate making by infrared laser exposure.

### [Planographic printing plate precursor]

Hereinafter, specific embodiments of the invention will be described, by taking application of the photosensitive composition to a recording layer of planographic printing plate precursor as an example. The planographic printing plate precursor has a support and a recording layer formed thereon, and may have additionally an undercoat layer, resin intermediate layer, backcoat layer, or the like according to applications. In the same way, the planographic printing plate precursor can be formed on by mounting the photosensitive composition on the support.

### [Recording layer]

A recording layer from the photosensitive composition according to the invention is formed by dissolving the components for the recording layer (the photosensitive composition according to the invention) in a solvent, thus forming a coating solution for recording layer, and applying the solution onto a suitable support. Other layers, including undercoat layer, resin intermediate layer, backcoat layer, and the like, can also be formed similarly.

Examples of the solvent in this case include ethylene dichloride, cyclohexanone, methyl ethyl ketone, methanol, ethanol, propanol, ethylene glycol monomethyl ether, 1-methoxy-2-propanol, 2-methoxyethyl acetate, 1-methoxy-2-propyl acetate, dimethoxyethane, methyl lactate, ethyl lactate, N,N-dimethylacetoamide, N,N-dimethylformamide, tetramethylurea, N-methylpyrrolidone, dimethylsulfoxide, sulfolane, γ-butyrolactone, and toluene. However, the solvent is not limited thereto. Moreover, these solvents may be used alone, or in a mixture form.

The concentration of the components for recording layer in the solvent (all solid matters including additives) is preferably 1 to 50% by weight.

In addition, a surfactant for improvement in coating property, for example, one of the fluorochemical surfactants described in JP-A No. 62-170950, may be added to the coating solution for recording layer. The preferable addition amount is 0.01 to 1% and still more preferably 0.05 to 0.5% by weight with respect to the total solid matters.

Various coating methods, for example, including bar coater coating, spin coating, spray coating, curtain coating, dip coating, air knife coating, blade coating, roll coating, and the like, may be used as the coating method.

The amount of the coat on the support obtained after application and drying (solid matter) may vary according to applications, but is generally, preferably 0.5 to 5.0 g/m² in the case of the recording layer for planographic printing plate precursors. Decrease in the coating amount leads to apparent increase in sensitivity but also to deterioration in the film properties of image-forming layer.

The recording layer may be a single layer or a layer in the multilayer structure.

### [Support]

The support used in the planographic printing plate precursor is a plate having dimensional stability. A plate satisfying required physical properties such as strength and flexibility can be used without any restriction. Examples thereof include paper, plastic (such as polyethylene, polypropylene or polystyrene)-laminated papers, metal plates (such as aluminum, zinc and copper plates), plastic films (such as cellulose biacetate, cellulose triacetate, cellulose propionate, cellulose lactate, cellulose acetate lactate, cellulose nitrate, polyethylene terephthalate, polyethylene, polystyrene, polypropylene, polycarbonate, and polyvinyl acetate films), and papers or plastic films on which, as described above, a metal is laminated or vapor-deposited.

The support is preferably a polyester film or an aluminum plate, and more preferably an aluminum plate, since an aluminum plate is superior in terms of dimensional stability and is also relatively inexpensive.

Preferable examples of the aluminum plate include a pure aluminum plate and alloy plates made of aluminum as a main component with a very small amount of other elements. A plastic film on which aluminum is laminated or vapor-deposited may also be used.

Examples of other elements contained in the aluminum alloys include silicon, iron, manganese, copper, magnesium, chromium, zinc, bismuth, nickel, and titanium. The content by percentage of different elements in the alloy is at most 10% by mass. A particularly preferable aluminum plate in the invention is a pure aluminum plate; however, since from the viewpoint of refining a completely pure aluminum cannot be easily produced, a very small amount of other elements may also be contained in the plate.

The aluminum plate used as the support is not specified in terms of the composition thereof. Thus, aluminum plates which are conventionally known can be appropriately used. The thickness of the aluminum plate used in the invention is from about 0.1 to 0.6 mm, preferably from 0.15 to 0.4 mm, and more preferably from 0.2 to 0.3 mm.

If necessary, prior to the surface-roughening treatment, the aluminum plate may optionally be subjected to degreasing treatment, in order to remove rolling oil or the like on the surface, with a surfactant, an organic solvent, an aqueous alkaline solution or the like.

The surface-roughening treatment of the aluminum surface can be performed by various methods such as a mechanical surface-roughening method, a method of dissolving and roughening the surface electrochemically, and a method of dissolving the surface selectively in a chemical manner.

Mechanical surface-roughening methods which can be used may be known methods, such as a ball polishing method, a brush polishing method, a blast polishing method or a buff polishing method. An electrochemical surface-roughening method may be a method of performing surface-roughening in an electrolyte of hydrochloric acid or nitric acid, by use of an alternating current or a direct current. As disclosed in JP-A No. 54-63902, a combination of the two kinds of methods may be used.

An aluminum plate whose surface is roughened as described above is if necessary subjected to alkali-etching treatment and neutralizing treatment. Thereafter, an anodizing treatment is optionally applied in order to improve the water holding capacity and wear resistance of the surface.

The electrolyte used in the anodizing treatment of the aluminum plate is any one selected from various electrolytes which can form a porous oxide film. Among which in general use are electrolytes of sulfuric acid, phosphoric acid, oxalic acid, chromic acid, or a mixed acid thereof. The concentration of the electrolyte may be appropriately decided depending on the kind of electrolyte selected.

Treatment conditions for anodization cannot be specified as a general rule since conditions vary depending on the electrolyte used; however; the following range of conditions are generally suitable: an electrolyte concentration of 1 to 80% by mass, a solution temperature of 5 to 70°C, a current density of 5 to 60 A/dm², a voltage of 1 to 100 V, and an electrolyzing time of 10 seconds to 5 minutes. If the amount of anodic oxide film is less than 1.0 g/m², printing resistance is inadequate or non-image portions of the planographic printing plate tend to become easily damaged and the so-called "blemish stains", resulting from ink adhering to damaged portions at the time of printing, are easily generated.

After the anodizing treatment, the surface of the aluminum is if necessary subjected to treatment for obtaining hydrophilicity. This securance of hydrophilicity treatment may be an alkali metal silicate (for example, an aqueous sodium silicate solution) method, as disclosed in U.S. Patent Nos. 2,714,066, 3,181,461, 3,280,734, and 3,902,734. In this method, the support is subjected to an immersing treatment or an electrolyzing treatment with an aqueous sodium silicate solution.

In addition, the following methods may also be used: a method of treating the support with potassium fluorozirconate, as disclosed in JP-B No. 36-22063, or with polyvinyl phosphonic acid, as disclosed in U.S. Patent Nos. 3,276,868, 4,153,461, and 4,689,272.

### [Undercoat layer]

In the planographic printing plate precursor of the present invention, if necessary, an undercoat layer may be formed between the support and the recording layer.

As components of the undercoat layer, various organic compounds can be used. Examples thereof include carboxymethylcellulose, dextrin, gum arabic, phosphonic acids having an amino group, such as 2-aminoethylphosphonic acid, organic phosphonic acids which may have a substituent, such as phenyl phosphonic acid, naphthylphosphonic acid, alkylphosphonic acid, glycerophosphonic acid, methylenediphosphonic acid and ethylenediphosphonic acid, organic phosphoric acids which may have a substituent, such as phenylphosphoric acid, naphthylphosphoric acid, alkylphosphoric acid and glycerophosphoric acid, organic phosphinic acids which may have a substituent, such as phenylphosphinic acid, naphthylphosphinic acid, alkylphosphinic acid and glycerophosphinic acid, amino acids such as glycine and β-alanine, and hydrochlorides of amines having a hydroxyl group, such as a hydrochloride of triethanolamine. These organic compounds may be used alone or in the form of a mixture made up of two or more thereof.

This organic undercoat layer may be formed by methods which can be described as follows: a method of applying onto the aluminum plate a solution wherein the above-mentioned organic compound is dissolved in water, or an organic solvent such as methanol, ethanol or methyl ethyl ketone, or a mixed solvent thereof and then drying the resultant aluminum plate, or a method of immersing the aluminum plate into a solution wherein the above-mentioned organic compound is dissolved in water, or an organic solvent such as methanol, ethanol or methyl ethyl ketone, or a mixed solvent thereof so as to adsorb the compound, washing the aluminum plate with water or the like, and then drying the resultant aluminum plate.

In the former method, the solution of the organic compound having a concentration of 0.05 to 10% by mass may be applied in various ways. In the latter method, the concentration of the organic compound in the solution is from 0.01 to 20%, preferably from 0.05 to 5%, the temperature for the immersion is from 20 to 90°C, preferably from 25 to 50°C, and the time taken for immersion is from 0.1 second to 20 minutes, preferably from 2 seconds to 1 minute.

The pH of the solution used in the above-mentioned methods can be adjusted into a range of 1 to 12 with a basic material such as ammonia, triethylamine or potassium hydroxide, or an acidic material such as hydrochloric acid or phosphoric acid. Moreover, a yellow dye may be added to the solution, in order to improve the tone reproducibility of the recording layer.

The amount of organic undercoat layer applied is suitably from 2 to 200 mg/m², preferably from 5 to 100 mg/m².

### [Resin intermediate layer]

The planographic printing plate precursor may have a resin intermediate layer formed as needed between the support and the recording layer (or, between the undercoat layer and the support if the undercoat layer has been formed).

Presence of the resin intermediate layer has advantages that it allows formation of a recording layer, i.e., an infrared ray-sensitive layer that becomes more soluble in alkaline developer by exposure, on the exposure surface or at a site closer thereto, improving the sensitivity thereof to the infrared laser, and at the same time, the resin intermediate layer, a polymer layer between the support and the infrared ray-sensitive layer, functions as a heat-insulating layer, prohibiting diffusion of the heat generated by exposure of infrared laser to the support, allowing more efficient use of the heat for image formation, and thus making the recording layer more sensitive.

In the unexposed region, the recording layer non-permeable into the alkaline developer seems to function as a protective layer for the resin intermediate layer, improving developing stability, providing images superior in color discrimination and stability over time.

In the exposed region, the components in the recording layer, which are set free from solubilization inhibition, become dissolved or dispersed in the developer rapidly and the resin intermediate layer consisting of an alkali-soluble polymer, which is readily soluble in the developer and present close to the support, dissolves rapidly without leaving residual layer or the like, improving the printing properties, for example, even when a less active developer or the like is used. Thus, the resin intermediate layer is useful in various ways.

### [Preparation of planographic printing plate precursor]

Plate making steps for the planographic printing plate precursor having respective layers formed as above (image exposure, development, and printing step) are next described below.

### (Light exposure)

Light sources for the beam used in image exposure are favorably, for example, light sources having an emission wavelength in the near-infrared to infrared regions, and particularly preferably, solid state lasers and semiconductor lasers.

When applied to a recording layer of planographic printing plate precursor, the photosensitive composition according to the invention does not cause deterioration in printing properties because of its superior post-exposure stability, even when the applied planographic printing plate precursor is not developed immediately after exposure but developed after a certain time. Thus, such a planographic printing plate precursor is useful, for example, when multiple planographic printing plate precursors stocked after exposure are processed together in an automatic developing machine, and shows such a printing properties that the images developed after a certain time are not inferior in quality to those immediately after exposure.

### (Development)

As the developer and replenisher for the planographic printing plate precursor wherein the photosensitive composition of the invention is used as its recording layer, aqueous solutions of a conventional alkali agent can be used.

Examples of the alkali agent include inorganic alkali salts such as sodium silicate, potassium silicate, trisodium phosphate, tripotassium phosphate, triammonium phosphate, disodium hydrogenphosphate, dipotassium hydrogenphosphate, diammonium hydrogenphosphate, sodium carbonate, potassium carbonate, ammonium carbonate, sodium hydrogencarbonate, potassium hydrogencarbonate, ammonium hydrogen carbonate, sodium borate, potassium borate, ammonium borate, sodium hydroxide, ammonium hydroxide, potassium hydroxide and lithium hydroxide; and organic alkali agents such as_monomethylamine, dimethylamine, trimethylamine, monoethylamine, diethylamine, triethylamine, monoisopropylamine, diisopropylamine, triisopropylamine, n-butylamine, monoethanolamine, diethanolamine, triethanolamine, monoisopropanolamine, diisopropanolamine, ethyleneimine, ethylenediamine, and pyridine. These alkali agents may be used alone or in combinations of two or more thereof.

Among these alkali agents, silicates such as sodium silicate and potassium silicate are particularly preferable for the developer. This is because the developing capacity of the developer can be controlled by adjusting the ratio between silicon oxide (SiO₂) and alkali metal oxide (M₂O), which are components of any one of the silicates, and by adjusting the concentrations thereof. For example, alkali metal silicates as described in JP-A No. 54-62004 or JP-B No. 57-7427 can be effectively used.

In a case where an automatic developing machine is used to perform development, an aqueous solution having a higher alkali intensity than that of the developer (or, replenisher) can be added to the developer. It is known that this makes it possible to treat a great number of photosensitive plates without recourse to replacing the developer in the developing tank over a long period of time. This replenishing manner is also preferably used in the invention.

If necessary, various surfactants or organic solvents can be incorporated into the developer and the replenisher in order to promote and suppress development capacity, disperse development scum, and enhance the ink-affinity of image portions of the printing plate.

Preferable examples of the surfactant include anionic, cationic, nonionic and amphoteric surfactants. If necessary, the following may be added to the developer and the replenisher: a reducing agent (such as hydroquinone, resorcin, a sodium or potassium salt of an inorganic acid such as sulfurous acid or hydrogen sulfite acid), an organic carboxylic acid, an antifoaming agent, and a water softener.

The printing plate developed with the developer and replenisher described above is subsequently subjected to treatments with washing water, a rinse solution containing a surfactant and other components, and a desensitizing solution containing gum arabic and a starch derivative. For after treatment following use of the photosensitive composition of the invention as a planographic printing plate precursor, various combinations of these treatments may be employed.

In recent years, automatic developing machines for printing plate precursors have been widely used in order to rationalize and standardize plate-making processes in the plate-making and printing industries. These automatic developing machines are generally made up of a developing section and a post-processing section, and include a device for carrying printing plate precursors, various treating solution tanks, and spray devices. These machines are machines for spraying respective treating solutions, which are pumped up, onto an exposed printing plate through spray nozzles, for development, while the printing plate is transported horizontally.

Recently, a method has also attracted attention in which a printing plate precursor is immersed in treating solution tanks filled with treating solutions and conveyed by means of in-liquid guide rolls. Such automatic processing can be performed while replenishers are being replenished into the respective treating solutions in accordance with the amounts to be treated, operating times, and other factors.

A so-called use-and-dispose processing manner can also be used, in which treatments are conducted with treating solutions which in practice have yet been used.

In cases where unnecessary image portions (for example, a film edge mark of an original picture film) are present on a planographic printing plate obtained by exposing-imagewise to light a planographic printing plate precursor to which the invention is applied, developing the exposed precursor, and subjecting the developed precursor to water-washing and/or rinsing and/or desensitizing treatment(s), unnecessary image portions can be erased.

The erasing is preferably performed by applying an erasing solution to unnecessary image portions, leaving the printing plate as it is for a given time, and washing the plate with water, as described in, for example, JP-B No. 2-13293. This erasing may also be performed by a method of radiating active rays introduced through an optical fiber onto the unnecessary image portions, and then developing the plate, as described in JP-A No. 59-174842.

### (Heating treatment (baking treatment))

The developed planographic printing plate thus obtained may be further coated with a desensitizing gum if desired before it is sent to the printing process; or the plate is additionally subjected to a baking treatment if desired for the purpose of obtaining planographic printing plates higher in printing durability. In particular, when the photosensitive composition according to the invention is applied to a recording layer of planographic printing plate precursor, a common baking treatment leads to drastic increase in printing durability, because the recording layer contains a novolak resin (A) having phenolic hydroxyl groups and thus is heat-crosslinkable.

It is preferable to treat the plate precursor with an affinitizing solution described in JP-B Nos. 61-2518 and 55-28062 and JP-A Nos. 62-31859 and 61-159655 before the baking treatment. The methods include application of the affinitizing solution onto the planographic printing plate with a sponge or cotton moistened therewith, application by immersing the printing plate into a bath filled with the affinitizing solution, and application by an automatic coater. Additionally, adjustment of the coating amount to uniformity by using a squeezee or a squeezee roller after application of the affinitizing solution leads to further preferable results.

The suitable amount of the affinitizing solution coated is generally 0.03 to 0.8 g/m² (as dry weight). Then, the planographic printing plate with the affinitizing solution applied may be dried as needed.

The planographic printing plat according to the invention is subsequently subjected to a heating treatment. The heating method is not particularly limited if it is effective in improving the printing durability, one of the advantageous effects of the invention by applying heat onto plate surface, and the examples thereof include methods of heating in a baking processor and others.

In the invention, among the heating methods above, preferable is a method of heating at high temperature in a baking processor (e.g. Baking Processor BP-1300, sold by Fuji Photo Film) or the like. The temperature and the period of the heating vary according to the kind of the components constituting the upper layer and the image-recording layer, but are preferably in the range of 150 to 300°C for 0.5 to 20 minutes and more preferably in the range of 180 to 270°C for 1 to 10 minutes.

The planographic printing plate after the baking treatment may be then subjected if needed to treatments commonly practiced in the art such as water washing and gumming, but if an affinitizing solution containing a water-soluble polymer compound or the like is used, so-called desensitizing treatments such as gumming and the like may be eliminated.

The planographic printing plates obtained after these treatments are then supplied to an offset printing machine or the like, wherein they are used for printing numerous papers.

### EXAMPLES

Hereinafter, the present invention will be described with reference to Examples, but it should be understood that the scope of the invention is not limited to these Examples.

### [Examples 1 to 12 and Comparative Examples 1 to 8]

### (Preparation of support)

Supporting plates were prepared in the following steps, using a JIS-A-1050 aluminium plate having a thickness of 0.3 mm.

### (a) Mechanical surface-roughening treatment

While a suspension of an abrasive agent (silica sand) having a specific gravity of 1.12 in water was supplied as an abrading slurry onto a surface of any one of the aluminum plates, the surface was mechanically roughened with rotating roller-form nylon brushes. The average grain size of the abrasive agent was 8 µm and the maximum grain size thereof was 50 µm. The material of the nylon brushes was 6·10-nylon, the length of bristles thereof was 50 mm, and the diameter of the bristles was 0.3 mm. The nylon brushes were each obtained by making holes in a stainless steel cylinder having a diameter of 300 mm and then planting bristles densely into the holes. The number of the used rotating brushes was three. The distance between the two supporting rollers (diameter: 200 mm) under each of the brushes was 300 mm. Each of the brush rollers was pushed against the aluminum plate until the load of a driving motor for rotating the brush became 7 kW larger than the load before the brush roller was pushed against the aluminum plate. The rotating direction of the brush was the same as the moving direction of the aluminum plate. The rotation speed of the brush was 200 rpm.

### (b) Alkali etching treatment

A 70°C aqueous solution of NaOH (NaOH concentration: 26% by mass, and aluminum ion concentration: 6.5% by mass) was sprayed onto the aluminum plate obtained in the above-mentioned manner to etch the aluminum plate, thereby dissolving the aluminum plate by 6 g/m². Thereafter, the aluminum plate was washed with water.

### (c) Desmutting treatment

The aluminum plate was subjected to desmutting treatment with a 30°C aqueous solution having a nitric acid concentration of 1% by mass (and containing 0.5% by mass of aluminum ions), which was sprayed, and then washed with water. The aqueous nitric acid solution used in the desmutting treatment was waste liquid derived from the step of conducting electrochemical surface-roughening treatment using alternating current in an aqueous nitric acid solution.

### (d) Electrochemical surface-roughening treatment

Alternating current having a frequency of 60 Hz was used to conduct electrochemical surface-roughening treatment continuously. The electrolyte used at this time was a 10.5 g/L solution of nitric acid in water (containing 5 g/L of aluminum ions), and the temperature thereof was 50°C. The wave of the used alternating current was a trapezoidal wave wherein the time TP until the current value was raised from zero to a peak was 0.8 msec, and the duty ratio of the current was 1:1. This trapezoidal wave alternating current was used, and a carbon electrode was set as a counter electrode to conduct the electrochemical surface-roughening treatment. Ferrite was used as an auxiliary anode. The used electrolyte bath was a radial cell type bath.

The density of the current was 30 A/dm² when the current was at the peak. The total amount of consumed electricity when the aluminum plate functioned as an anode was 220 C/dm². Five percent of the current sent from a power source was allowed to flow into the auxiliary anode.

Thereafter, the aluminum plate was washed with water.

### (e) Alkali etching treatment

An aqueous solution having a caustic soda of 26% by mass and an aluminum ion concentration of 6.5% by mass was sprayed onto the aluminum plate to etch the plate at 32°C so as to dissolve the aluminum plate by 0.20 g/m², thereby removing smut components made mainly of aluminum hydroxide and generated when the alternating current was used to conduct the electrochemical surface-roughening treatment in the previous step, and further dissolving edges of formed pits so as to be made smooth. Thereafter, the aluminum plate was washed with water.

### (f) Desmut treatment

The aluminum plate was subjected to desmutting treatment with a 30°C aqueous solution having a nitric acid concentration of 15% by mass (and containing 4.5% by mass of aluminum ions), which was sprayed, and then washed with water. The aqueous nitric acid solution used in the desmutting treatment was waste liquid derived from the step of conducting the electrochemical surface-roughening treatment using the alternating current in the aqueous nitric acid solution.

### (g) Electrochemical surface-roughening treatment

Alternating current having a frequency of 60 Hz was used to conduct electrochemical surface-roughening treatment continuously. The electrolyte used at this time was a 7.5 g/L solution of hydrochloric acid in water (containing 5 g/L of aluminum ions), and the temperature thereof was 35°C. The wave of the alternating current was a rectangular wave. A carbon electrode was set as a counter electrode to conduct the electrochemical surface-roughening treatment. Ferrite was used as an auxiliary anode. The used electrolyte bath was a radial cell type bath.

The density of the current was 25 A/dm² when the current was at the peak. The total amount of consumed electricity when the aluminum plate functioned as an anode was 50 C/dm².

Thereafter, the aluminum plate was washed with water.

### (h) Alkali etching treatment

An aqueous solution having a caustic soda of 26% by mass and an aluminum ion concentration of 6.5% by mass was sprayed onto the aluminum plate to etch the plate at 32°C so as to dissolve the aluminum plate by 0.10 g/m², thereby removing smut components made mainly of aluminum hydroxide and generated when the alternating current was used to conduct the electrochemical surface-roughening treatment in the previous step, and further dissolving edges of formed pits so as to be made smooth. Thereafter, the aluminum plate was washed with water.

### (i) Desmutting treatment

The aluminum plate was subjected to desmutting treatment with a 60°C aqueous solution having a sulfuric acid concentration of 25% by mass (and containing 0.5% by mass of aluminum ions), which was sprayed, and then washed with water.

### (j) Anodizing treatment

As electrolytes, sulfuric acid was used. The electrolytes were each an electrolyte having a sulfuric acid concentration of 170 g/L (and containing 0.5% by mass of aluminum ions), and the temperature thereof was 43°C. Thereafter, the support was washed with water.

The current densities were each about 30 A/dm². The final amount of the oxidation film was 2.7 g/m².

### <Support A>

The above steps (a) to (j) were successively performed and the etching amount in step (e) was set to 3.4 g/m², so as to form a support A.

### <Support B>

The above-mentioned steps other than steps (g), (h) and (i) were successively performed to form a support B.

### <Support C>

The above-mentioned steps other than steps (a), (g), (h) and (i) were successively performed to form a support C.

### <Support D>

The above-mentioned steps other than the steps (a), (g), (h) and (i) were successively performed, and the total amount of consumed electricity in step (g) was set to 450 C/dm², to form a support D.

The supports A, B, C and D obtained in the above-mentioned manner were subjected to the following treatment to make the support surface hydrophilic and apply undercoat to the support.

### (k) Treatment with alkali metal silicate

Each of the aluminum supports A to D obtained in the above-mentioned manner was immersed into a treatment tank containing a 30°C aqueous solution of #3 sodium silicate (concentration of sodium silicate: 1% by mass) for 10 seconds to subject the support to treatment with the alkali metal silicate (silicate treatment). Thereafter, the support was washed with water. The amount of the silicate adhering at this time was 3.5 mg/m².

### (Undercoat treatment)

An undercoat solution having the following composition was applied onto each of the aluminum supports treated with the alkali metal silicate, which supports were obtained in the above-mentioned manner, and the resultant was dried at 80°C for 15 seconds. The applied amount of solid contents after the drying was 18 mg/m².

### <Undercoat solution composition>

- Polymer compound having a structure illustrated below 0.3 g
- Methanol 100 g
- Water 1.0 g

The photosensitive composition of the invention is evaluated by evaluating planographic printing plate precursors employing the photosensitive composition of the invention in the recording layer.

### [Evaluation method]

The planographic printing plate precursors were stored for 5 days under conditions of a temperature of 25°C and a relative humidity of 50%, and a test pattern was formed imagewise on each of the planographic printing plate precursors using TRENDSETTER 3244 VX (trademark) manufactured by Creo at a beam intensity of 10.0 W and a drum rotational velocity of 125 rpm.

Then, the planographic printing plate precursors were developed at a constant liquid temperature of 30°C and a development period of 25 seconds in PS PROCESSOR 900H manufactured by Fuji Photo Film Co. Ltd., that contained a diluted solution of the alkaline developer A or B, having the compositions described below, of which the electrical conductivity was adjusted by changing the content of water and thus the dilution rate in the alkali developer. Then, using planographic printing plates, which were developed with a developer having an intermediate developer activity between the maximum and minimum electrical conductivities of the developer that provided good development without dissolution of image areas and without stains and discoloration due to residues of a poorly developed photosensitive layer in non-image areas, printing was conducted on MITSUBISHI DIAMOND-TYPE F2 PRINTER (manufactured by Mitsubishi Heavy Industries., Ltd.) with DIC-GEOS (s) crimson ink to obtain 10,000 prints, and then staining on a blanket was visually evaluated.

Criteria for the evaluation were:
A: no staining,
B: little staining, and
C: significant staining.

### <Composition of alkaline developer A>

- SiO₂·K₂O[K₂O/SiO₂=1/1 (molar ratio)] 4.0% by weight
- Citric acid 0.5% by weight
- Polyethylene glycol laurylether 0.5% by weight
   (weight-average molecular weight: 1,000)
- Water 95.0% by weight

### <Composition of alkaline developer B>

- D-sorbit 2.5% by weight
- Sodium hydroxide 0.85% by weight
- Polyethylene glycol laurylether 0.5% by weight
   (weight-average molecular weight: 1,000)
- Water 96.15% by weight

### Examples

### [Examples 1 to 3, Comparative Examples 1 and 2]

The coating solution for the first layer (lower layer), having the composition described below, was applied by using a wire bar onto the support A to give a coating amount of 0.95 g/m² after the support A was dried in a drying oven at 150°C for 60 seconds.

The coating solution for the second layer (upper layer), having the composition described below, was then applied by a wire bar onto the support having the undercoat layer thus obtained. After application, the support A was dried in a drying oven at 130°C for 90 seconds, to produce positive-type planographic printing plate precursors of Examples 1 to 3 and Comparative Examples 1 and 2 respectively having total coating amounts of 1.25 g/m².

### <Coating solution for first layer (lower layer)>

- Copolymer 1 (prepared as described below) 1.833 g
- Cyanine dye A (having the structure below) 0.098 g
- 2-Mercapto-5-methylthio-1,3,4-thiadiazole 0.030 g
- Cis-Δ⁴-tetrahydrophthalic acid anhydride 0.100 g
- 4,4'-Sulfonyl diphenol 0.090 g
- p-Toluenesulfonic acid 0.008 g
- Ethyl violet having 6-hydroxynaphthalenesulfonic acid 0.100 g
   as the counter anion
- 3-Methoxy-4-diazodiphenylamine hexafluorophosphate 0.030 g
- Fluorochemical surfactant 0.035 g
   (Megafac F-780 (trademark), manufactured by Dainippon Ink and Chemicals, Inc.)
- Methylethylketone 26.6 g
- 1-Methoxy-2-propanol 13.6 g
- γ-Butylolactone 13.8 g

### <Preparation of copolymer 1>

After stirring, 31.0 g (0.36 mole) of methacrylic acid, 39.1 g (0.36 mole) of ethyl chloroformate, and 200 ml of acetonitrile were placed in a 500 ml three-necked flask equipped with a stirrer, a condenser tube, and a dropping funnel, and the mixture was stirred while being cooled in an ice water bath. 36.4 g (0.36 mole) of triethylamine was added to the mixture dropwise via a dropping funnel over the period of approximately 1 hour. After the dropwise addition, the ice water bath was removed and the mixture was stirred at room temperature for 30 minutes.

51.7 g (0.30 mole) of p-aminobenzenesulfonamide was added to the reaction mixture, and the resulting mixture was then stirred in an oil bath while heated at 70°C for 1 hour. After completion of the reaction, the mixture was poured into 1 liter of water while stirring, and the mixture was stirred additionally for 30 minutes. The precipitate was collected by filtration of the mixture and re-suspended in 500 ml of water, and the solid obtained by filtration of this slurry was dried, to give white a solid of N-(p-aminosulfonylphenyl)methacrylamide (yield: 46.9 g).

Then, 4.61 g (0.0192 mole) of N-(p-aminosulfonylphenyl) methacrylamide, 2.58 g (0.0258 mole) of ethyl methacrylate, 0.80 g (0.015 mole) of acrylonitrile, and 20 g of N,N-dimethylacetamide were placed in a 20 ml three-necked flask equipped with a stirrer, a condenser tube, and a dropping funnel, and the mixture was stirred while heated in a hot water bath at 65°C.

To the mixture, 0.15 g of 2,2'-azobis(2,4-dimethylvaleronitrile) (brand name: "V-65", manufactured by Wako Pure Chemical Industries) was added as a polymerization initiator, and the mixture was stirred at 65°C under a nitrogen stream for 2 hours.

Further, a mixture of 4.61 g of N-(p-aminosulfonylphenyl) methacrylamide, 2.58 g of methyl methacrylate, 0.80 g of acrylonitrile, 20 g of N,N-dimethylacetamide and 0.15 g of "V-65" was added dropwise via a dropping funnel to the reaction mixture over 2 hours. After dropwise addition, the mixture obtained was additionally stirred at 65°C for 2 hours.

After completion of the reaction, 40 g of methanol was added to the mixture; the resulting mixture was cooled and poured into 2 liters of water while stirring; the resulting mixture was stirred for 30 minutes; and the precipitate obtained by filtration was dried to give 15 g of a white solid. The weight-average molecular weight (polystyrene standard) of the particular copolymer 1 as determined by gel-permeation chromatography was 54,000.

### <Coating solution for second layer (upper layer) >

- Copolymer from ethyl methacrylate 0.040 g
   and 2-methacryloyloxyethylsuccinic acid
   (molar ratio: 75 : 25, weight-average molecular weight: 70,000)
- Phenol cresol-formaldehyde novolak 0.400 g
   (phenol : m-cresol : p-cresol = 50 : 30 : 20,
   weight average molecular weight: 8800)
- Specific sulfonium salt or comparative onium salt 0.1 g
- Cyanine dye A (having the structure above) 0.015 g
- Ethyl violet having 6-hydroxynaphthalenesulfonic acid 0.012 g
   as the counter anion
- Fluorochemical surfactant 0.022 g
   (Megafac F-780 (trademark), manufactured by Dainippon Ink and Chemicals, Inc.)
- Methylethylketone 13.1 g
- 1-Methoxy-2-propanol 6.79 g

It should be noted that the numbers given in Table 1 below for the respective specific sulfonium salts correspond to the compound numbers of the exemplary compounds listed above.

**Table 1**

| | Sulfonium salt | Hammett value | Log P | Anti-scumming property |
|---|---|---|---|---|
| Example 1 | 68 | 0.69 | -1.312 | A |
| Example 2 | 77 | 0.69 | 0.799 | A |
| Example 3 | structure shown below | 0.69 | 2.609 | B |
| Comp. Ex. 1 | 28 (below) | 0 | 4.233 | C |
| Comp. Ex. 2 | 13 (below) | 0 | -0.146 | C |

As can be seen from Table 1, the planographic printing plate precursors of Examples 1 to 3 employing the photosensitive composition of the invention in the recording layer accomplishes improvement in the anti-scumming property. On the other hand, the planographic printing plate precursors of Comparative Examples 1 and 2,
where compounds having cation moiety with smaller Hammett values are employed, exhibit significantly poorer anti-scumming property. Further, comparing Examples 1 and 2 and Example 3, it is confirmed that a particularly remarkable effect is obtained when a sulfonium salt having a cation structure with a smaller Hammett value, as well as an anion moiety with log P within the preferable range, is used.

### [Examples 4 to 6, Comparative Examples 3 and 4]

The coating solution for the first layer (lower layer), having the composition described below, was applied by using a wire bar onto the support C to give a coating amount of 0.60 g/m² after the support C was dried in a drying oven at 120°C for 90 seconds.

The coating solution for the second layer (upper layer), having the composition described below, was then applied by a wire bar onto the support having the undercoat layer thus obtained. After application, the support C was dried in a drying oven at 120°C for 90 seconds, to produce positive-type planographic printing plate precursors of Examples 4 to 6 and Comparative Examples 3 and 4 respectively having total coating amounts of 1.35 g/m².

### <Coating solution for first layer (lower layer)>

- Copolymer 1 2.200 g
- Cyanine dye A (having the structure above) 0.098 g
- 2-Mercapto-5-methylthio-1,3,4-thiadiazole 0.030 g
- Cis-Δ⁴-tetrahydrophthalic acid anhydride 0.100 g
- 4,4'-Sulfonyl diphenol 0.090 g
- p-Toluenesulfonic acid 0.008 g
- Ethyl violet having 6-hydroxynaphthalenesulfonic acid 0.100 g
   as the counter anion
- 3-Methoxy-4-diazodiphenylamine hexafluorophosphate 0.030 g
- Fluorochemical surfactant 0.035 g
   (Megafac F-780 (trademark), manufactured by Dainippon Ink and Chemicals, Inc.)
- Methylethylketone 26.6 g
- 1-Methoxy-2-propanol 13.6 g
- Dimethyl sulfoxide 13.8 g

### <Coating solution for second layer (upper layer) >

- Copolymer from ethyl methacrylate 0.040 g
   and 2-methacryloyloxyethylsuccinic acid
   (molar ratio: 70 : 30, weight-average molecular weight: 88,000)
- Phenol cresol-formaldehyde novolak 0.250 g
   (phenol : m-cresol : p-cresol = 30 : 50 : 20,
   weight average molecular weight: 7700)
- Specific sulfonium salt or comparative onium salt compound 0.02 g
- Cyanine dye A (having the structure above) 0.015 g
- Fluorochemical surfactant 0.022 g
   (Megafac F-780 (trademark), manufactured by Dainippon Ink and Chemicals, Inc.)
- Methylethylketone 13.1 g
- 1-Methoxy-2-propanol 6.79 g

### <Evaluation of Examples 4 to 6 and Comparative Examples 3 and 4>

The resulting planographic printing plate precursors of Examples 4 to 6 and Comparative Examples 3 and 4 were respectively evaluated in the same manner as in Example 1. The developer B was used for developing the planographic printing plate precursors. Results are shown in Table 2.

It should be noted that the numbers given in Table 2 below for the respective specific sulfonium salts correspond to the compound numbers of the exemplary compounds listed above.

**Table 2**

| | Sulfonium salt | Hammett value | Log P | Anti-scumming property |
|---|---|---|---|---|
| Example 4 | 68 | 0.69 | -1.312 | A |
| Example 5 | 72 | 0.69 | -1.292 | A |
| Example 6 | Structure shown below | 0.69 | 2.609 | B |
| Comp. Ex. 3 | 28 | 0 | 4.233 | C |
| Comp. Ex. 4 | 13 | 0 | -0.146 | C |

As can be seen from Table 2, comparing with the planographic printing plate precursors of Comparative Examples, the planographic printing plate precursors of Examples 4-6 accomplishes improvement in the anti-scumming property, as in Examples 1 to 3. From this point, it is found that, even if components of the photosensitive layer are varied, the planographic printing plate precursors employing the photosensitive composition of the invention in the recording layer exhibit the same excellent effect.

### [Examples 7 to 9, Comparative Examples 5 and 6]

The coating solution for the first layer (lower layer), having the composition described below, was applied by using a wire bar onto the support D to give a coating amount of 0.81 g/m² after the support D was dried in a drying oven at 150°C for 60 seconds.

The coating solution for the second layer (upper layer), having the composition described below, was then applied by a wire bar onto the support having the undercoat layer thus obtained. After application, the support D was dried in a drying oven at 120°C for 90 seconds, to produce positive-type planographic printing plate precursors of Examples 7 to 9 and Comparative Examples 5 and 6 respectively having total coating amounts of 1.1 g/m².

### <Coating solution for first layer (lower layer)>

- Copolymer 1 above 2.133 g
- Cyanine dye A (having the structure above) 0.098 g
- Cis-Δ⁴-tetrahydrophthalic acid anhydride 0.110 g
- 4,4'-Sulfonyl diphenol 0.090 g
- p-Toluenesulfonic acid 0.008 g
- Ethyl violet having 6-hydroxynaphthalenesulfonic acid 0.100 g
   as the counter anion
- 3-Methoxy-4-diazodiphenylamine hexafluorophosphate 0.030 g
- Fluorochemical surfactant 0.035 g
   (Megafac F-780 (trademark), manufactured by Dainippon Ink and Chemicals, Inc.)
- Methylethylketone 26.6 g
- 1-Methoxy-2-propanol 13.6 g
- γ-Butylolactone 13.8 g

### <Coating solution for second layer (upper layer) >

- Copolymer from ethyl methacrylate 0.0350 g
   and 2-methacryloyloxyethylsuccinic acid
   (molar ratio: 65 : 35, weight-average molecular weight: 78,000)
- Cresol-formaldehyde novolak 0.300 g
   (m-cresol : p-cresol = 60 : 40,
   weight average molecular weight: 4100)
- Specific sulfonium salt or comparative onium salt compound 0.0150 g
- Cyanine dye A (having the structure above) 0.015 g
- Fluorochemical surfactant 0.022 g
   (Megafac F-780 (trademark), manufactured by Dainippon Ink and Chemicals, Inc.)
- Methylethylketone 13.1 g
- 1-Methoxy-2-propanol 6.79 g

### <Evaluation of Examples 7 to 9 and Comparative Examples 5 and 6>

The resulting planographic printing plate precursors were evaluated in the manner described above. The developer A was used for developing the planographic printing plate precursors. Results are shown in Table 3.

The numbers given in Table 3 below for the respective specific sulfonium salts correspond to the compound numbers of the exemplary compounds listed above.

**Table 3**

| | Sulfonium salt | Hammett value | Log P | Anti-scumming property |
|---|---|---|---|---|
| Example 7 | 75 | 0.69 | -0.707 | A |
| Example 8 | 72 | 0.69 | -1.292 | A |
| Example 9 | structure shown below | 0.69 | 2.609 | B |
| Comp. Ex. 5 | 28 | 0 | 4.233 | C |
| Comp. Ex. 6 | 13 | 0 | -0.146 | C |

As can be seen from Table 3, the planographic printing plate precursors of Examples 7 to 9 accomplished improvement in the anti-scumming property. [Examples 10 to 12, Comparative Examples 7 and 8]

The image forming layer coating solution having the composition described below was applied onto the support D, and the support D was dried at 120°C for 90 seconds to form the image forming layer. Thus, planographic printing plate precursors of Examples 10 to 12 and Comparative Examples 7 and 8 were obtained. A dry coating amount was 1.60 g/m².

### < Image forming layer coating solution >

- Phenol cresol-formaldehyde novolak 1.0 g
   (phenol : m-cresol : p-cresol = 50 : 30 : 20,
   weight average molecular weight: 6500)
- Specific sulfonium salt or comparative onium salt compound 0.05 g
- Cyanine dye A (having the structure above) 0.05 g
- Dye, Victoria Pure Blue BOH, 0.01 g
   having an 1-naphthalenesulfonate anion as the counter anion
- Fluorochemical surfactant 0.05 g
   (Megafac F-177 (trademark), manufactured by Dainippon Ink and Chemicals, Inc.)
- Methylethylketone 9.0 g
- 1-Methoxy-2-propanol 9.0 g

### <Evaluation of Examples 10 to 12 and Comparative Examples 7 and 8>

The resulting planographic printing plate precursors of Examples 10 to 12 and Comparative Examples 7 and 8 were respectively evaluated in the same manner as in Example 1. The developer A was used for developing the planographic printing plate precursors. Results are shown in Table 4.

The numbers given in Table 4 below for the specific sulfonium salt correspond to the compound numbers of the exemplary compounds listed above.

**Table 4**

| | Sulfonium salt | Hammett value | Log P | Anti-scumming property |
|---|---|---|---|---|
| Example 10 | 76 | 0.69 | -0.935 | A |
| Example 11 | 72 | 0.69 | -1.292 | A |
| Example 12 | structure shown below | 0.69 | 2.609 | B |
| Comp. Ex. 7 | 28 | 0 | 4.233 | C |
| Comp. Ex. 8 | 13 | 0 | -0.146 | C |

As can be seen from Table 4, the planographic printing plate precursors of Examples 10 to 12 accomplishes improvement in the anti-scumming property.

Further, comparing Examples 1 to 3 and Examples 10 to 12, it is confirmed that the planographic printing plate precursors employing the photosensitive composition of the invention in the recording layer exhibit the same excellent effect of the invention, regardless of the recording layer being single-layered or multi-layered.

## Claims

1. A positive-type photosensitive composition comprising:
a novolak resin (A);
an infrared absorbing agent (B); and
a compound having a triarylsulfonium salt structure (C) in which the sum of the Hammett values of substituents bonded to aryl skeletons is greater than 0.46.

2. A positive-type photosensitive composition according to Claim 1, wherein the compound having a triarylsulfonium salt structure (C) contains a triarylsulfonium cation in which the sum of the Hammett values of substituents bonded to aryl skeletons is greater than 0.46 and an anion having a hydrophilicity/hydrophobicity parameter log P less than 2.

3. A positive-type photosensitive composition according to Claim 1, wherein the compound having a triarylsulfonium salt structure (C) contains a triarylsulfonium cation in which the sum of the Hammett values of substituents bonded to aryl skeletons is greater than 0.46 and an anion having a hydrophilicity/hydrophobicity parameter log P of -1 to 1.

4. A positive-type photosensitive composition according to Claim 1, wherein the compound having a triarylsulfonium salt structure (C) is a compound in which the sum of the Hammett values of substituents bonded to aryl skeletons is greater than 0.60.

5. A positive-type photosensitive composition according to Claim 1, wherein the compound having a triarylsulfonium salt structure (C) is substituted on each of the three aryl skeletons by Cl.

6. A positive-type planographic printing plate precursor comprising:
a hydrophilic support;
a lower layer containing a water-insoluble and alkali-soluble resin formed on the support; and
an image recording layer containing a positive-type photosensitive composition according to Claim 1 formed on the lower layer.

7. A positive-type planographic printing plate precursor comprising:
a hydrophilic support;
a lower layer containing a water-insoluble and alkali-soluble resin formed on the support; and
an image recording layer containing a positive-type photosensitive composition according to Claim 2 formed on the lower layer.

## Patentansprüche

1. Fotoempfindliche Zusammensetzung vom Positivtyp, umfassend:
ein Novolakharz (A);
einen Infrarotabsorber (B); und
eine Verbindung mit einer Triarylsulfoniumsalzstruktur (C), worin die Summe der Hammett-Werte der Substituenten, die an Arylgerüste gebunden sind, größer als 0,46 ist.

2. Fotoempfindliche Zusammensetzung vom Positivtyp gemäß Anspruch 1, worin die Verbindung mit einer Triarylsulfoniumsalzstruktur (C) ein Triarylsulfoniumkation enthält, worin die Summe der Hammett-Werte der Substituenten, die an Arylgerüste gebunden sind, größer als 0,46 ist und ein Anion einen Hydrophilizitäts/Hydrophobizitäts-Parameter log P von weniger als 2 aufweist.

3. Fotoempfindliche Zusammensetzung vom Positivtyp gemäß Anspruch 1, worin die Verbindung mit einer Triarylsulfoniumsalzstruktur (C) ein Triarylsulfoniumkation enthält, worin die Summe der Hammett-Werte der Substituenten, die an Arylgerüste gebunden sind, größer als 0,46 ist und ein Anion einen Hydrophilizitäts/Hydrophobizitäts-Parameter log P von -1 bis 1 aufweist.

4. Fotoempfindliche Zusammensetzung vom Positivtyp gemäß Anspruch 1, worin die Verbindung mit einer Triarylsulfoniumsalzstruktur (C) eine Verbindung ist, in der die Summe der Hammett-Werte der Substituenten, die an Arylgerüste gebunden sind, größer als 0,60 ist.

5. Fotoempfindliche Zusammensetzung vom Positivtyp gemäß Anspruch 1, worin die Verbindung mit einer Triarylsulfoniumsalzstruktur (C) an jedem der drei Arylgerüste mit Cl substituiert ist.

6. Flachdruckplattenvorläufer vom Positivtyp, umfassend:
einen hydrophilen Träger;
eine auf dem Träger gebildete untere Schicht, die ein wasserunlösliches und alkalilösliches Harz enthält; und
eine auf der unteren Schicht gebildete Bildaufzeichnungsschicht, die eine fotoempfindliche Zusammensetzung vom Positivtyp gemäß Anspruch 1 enthält.

7. Flachdruckplattenvorläufer vom Positivtyp, umfassend:
einen hydrophilen Träger;
eine auf dem Träger gebildete untere Schicht, die ein wasserunlösliches und alkalilösliches Harz enthält; und
eine auf der unteren Schicht gebildete Bildaufzeichnungsschicht, die eine fotoempfindliche Zusammensetzung vom Positivtyp gemäß Anspruch 2 enthält.

## Revendications

1. Composition photosensible de type positif comprenant :
une résine novolak (A) ;
un agent d'absorption infrarouge (B) ; et
un composé ayant une structure de sel triarylsulfonium (C) dans lequel la somme des valeurs de Hammett de substituants liés à des squelettes aryles est supérieure à 0,46.

2. Composition photosensible de type positif selon la revendication 1, dans laquelle le composé ayant une structure de sel triarylsulfonium (C) contient un cation triarylsulfonium dans lequel la somme des valeurs de Hammett de substituants liés à des squelettes aryles est supérieure à 0,46 et un anion ayant un paramètre d'hydrophilicité / hydrophobicité log P inférieur à 2.

3. Composition photosensible de type positif selon la revendication 1, dans laquelle le composé ayant une structure de sel triarylsulfonium (C) contient un cation triarylsulfonium dans lequel la somme des valeurs de Hammett de substituants liés à des squelettes aryles est supérieure à 0,46 et un anion ayant un paramètre d'hydrophilicité / hydrophobicité log P de - 1 à 1.

4. Composition photosensible de type positif selon la revendication 1, dans laquelle le composé ayant une structure de sel triarylsulfonium (C) est un composé dans lequel la somme des valeurs de Hammett de substituants liés à des squelettes aryles est supérieure à 0,60.

5. Composition photosensible de type positif selon la revendication 1, dans laquelle le composé ayant une structure de sel triarylsulfonium (C) est substitué sur chacun des trois squelettes aryles par Cl.

6. Précurseur de plaque d'impression planographique de type positif comprenant :
un support hydrophile ;
une couche inférieure contenant une résine insoluble dans l'eau et soluble dans l'alcali, formée sur le support ; et
une couche d'enregistrement d'image contenant une composition photosensible de type positif selon la revendication 1 formée sur la couche inférieure.

7. Précurseur de plaque d'impression planographique de type positif comprenant :
un support hydrophile ;
une couche inférieure contenant une résine insoluble dans l'eau et soluble dans l'alcali, formée sur le support ; et
une couche d'enregistrement d'image contenant une composition photosensible de type positif selon la revendication 2 formée sur la couche inférieure.
